

July 25, 1950

L. F. ROGERS ET AL

2,516,647

METHOD OF MAKING CLOSURE ELEMENTS

Filed May 13, 1946



INVENTORS  
LOUIS F. ROGERS  
MICHAEL S. EBERT  
BY

Mason, Parker, Diller & Stewart,  
ATTORNEYS

## UNITED STATES PATENT OFFICE

2,516,647

## METHOD OF MAKING CLOSURE ELEMENTS

Louis F. Rogers and Michael S. Ebert, Wilmington, Del., assignors to Continental Can Company, Inc., New York, N. Y., a corporation of New York

Application May 13, 1946, Serial No. 669,450

5 Claims. (Cl. 113—80)

1

In the preparation of container closure elements such as ends and crown seals, it has been the practice to employ an elastic liner for sealing the element to the container. For example, crown seals have been made with cork cushion liners with or without a central spot of aluminum foil, or with cushioning and sealing liners of natural rubber or like composition which was preformed and then inserted or was deposited in the formed crown shell as a fluid and then dried in place; wherewith the practice was first to punch and form a metal sheet into crown shells and then by subsequent operations adhesively apply the liners into the shells. Another proposal has been to print a metal sheet with disks or rings of thermo-adhesive substance and then punch and form the shells in the cold, then heat to adhesiveness, and then apply the liners.

According to the present invention, closure elements are prepared by printing the blank with a material which itself provides cushioning and sealing, in individually thin deposits which are successively made until the desired total thickness is obtained, and thereafter punching and forming the closure elements with the cushion seal already present on the blank.

In the accompanying drawing;

Figure 1 is a sectional view, on a greatly enlarged scale, of a metal sheet having a lithographed coating on its lower face;

Figure 2 is a corresponding view, showing the printing of a first cushion deposit on such a sheet;

Figure 3 is a corresponding view showing the printing of a second deposit;

Figure 4 is a corresponding view showing the sheet with three successive deposits thereon;

Figure 5 is a view, on the same scale, through a crown seal made in accordance with this invention;

Figure 6 is a perspective view on a smaller scale, showing part of a large sheet having a multiplicity of deposited areas thereon;

Figure 7 is a flow diagram, indicating the steps of a preferred method of operation.

In this illustrative practice of the invention, a flat blank sheet 10 (Figure 1) of metal, such as tin plate, is printed at the side which is later to provide the exposed surface of the cap, with the usual identifying and surfacing matter in the usual ways, these lithographed coatings 11 then

being baked in the usual fashion. The sheet is then subjected to a succession of further applying operations at its other face, employing a composition of the following formulation:

|                         | Parts by weight |
|-------------------------|-----------------|
| Artificial rubber (GRS) | 100             |
| Zinc oxide              | 5               |
| Sulphur                 | 1               |
| Vulcanizing agent       | 8               |
| Paraffin                | 20              |
| Clay                    | 250             |
| Titanium oxide          | 20              |
| Xylool                  | 800             |

- 15 2) The first applying operation deposits (Figure 2) a thin film 12 of this fluid material over an area of the blank which in size and shape corresponds to the inner end surface of the crown shell to be formed, covering this area entirely.
- 20 In practice, each sheet of metal (Figure 6) provides materials for several hundred blank crown shells and accordingly simultaneous application is made for these individual crown shells, locating each circle of deposit on the inner face but 25 in alignment with the lithographed identifying matter which has been placed on the outer face. A preferred manner of applying is by use of a silk screen printing stencil with impermeable portions 14, wherewith the circular deposits 12, at 30 points of the sheet corresponding to the location of the permeable screen portions 15 in the stencil, are produced by the delivery through untreated parts of the screen in the usual manner of silk screen printing. The sheet is then dried, where- 35 with the localized deposits 12 provide adhesive films having a thickness of about eight one-thousandths of an inch. The sheet is then subjected to further applying operations, in which the successive stencils with impermeable portions 16, 17 and annular permeable portions 18 deliver annular deposits 20, 21 along the outer periphery of the initial circular deposit, with a radial dimension corresponding to the dimension of the lip of the container which is to be closed by 40 the crown seal. Each successive application is dried before the next is applied, so that an annular structure is built up; these applications illustratively have individual thicknesses about eight one-thousandths of an inch after drying. 45 The same composition as above is employed. The 50

total thickness of the three layers of deposit (Figure 4) being the first or circular deposit 12 and two subsequent annular deposits 20, 21, is about twenty-five thousandths of an inch. The deposit should be cured before punching the crown seals therefrom. The curing or vulcanizing operation may be performed successively upon each of the layers as deposited in succession to the drying operation; or the curing can be effected upon a number of layers, or even upon all layers, at a single vulcanizing operation. It is presently preferred (diagram with legends Figure 7) to dry each layer individually before applying the next, and to employ the vulcanizing heat only after the total deposit has been effected. The curing can be accomplished by passing the printed sheets through an oven, e. g. on a moving conveyor, wherewith to heat them to a temperature of 240 degrees F. for thirty minutes, wherewith the material becomes vulcanized and fixed in its properties. Other time-temperature conditions can be used, as known in the art: care being taken to avoid employing excessive heating with mixtures which may be harmed thereby, as for example when very light colors are being printed, the temperature of exposure should be not over 260 degrees F. to prevent color-darkening.

When the last deposit has been completed and cured, the sheet is fed in the usual manner into a blanking and forming press, which has its die recesses and punches aligned with the locations of the identifying matter at the outer face for the crown shell and the above deposits at the inner face, and crown shells are now stamped and formed (note legend in Figure 7) to provide them the usual crimped skirts. The above composition adheres to the metal, and the output from the punch press is a bulk group of the formed crown shells (Figure 5) each having a multiple coating of the aforesaid material and structure at its interior, along with the residual scrap of the sheet.

These crown shells (Figure 3) have the usual body 10a and crimped skirt 10b, with the external lithographed matter 11 and the internal circular deposit 12 upon which are the two successive annular deposits 20, 21 located ready to engage the lip of a bottle, can, etc. They are now ready for application to bottles, cans, etc. by the usual sealing or crimping devices.

The artificial rubber employed in the above illustrative practice was the material available on the market under the name GR-S and is so called in "Specifications for Government Synthetic Rubbers" issued by Reconstruction Finance Corporation, Office of Rubber Reserve, and effective January 1, 1947. The material is a copolymer of butadiene and styrene to which approximately 1.25% of a standard rubber antioxidant has been added during manufacture: of the hydrocarbon present, approximately 23.5% by weight is derived from styrene.

Other types of butadiene-styrene copolymer rubber, natural rubber, butyl rubber and mixtures of natural and synthetic rubbers, may be employed, provided that the same is capable of forming a homogeneous and essentially compatible mixture with the paraffin and is capable upon the said vulcanization of producing a mass of elastically yielding characteristic.

The vulcanizing agent employed can be of the type commercially used with rubber compositions: in general, the accelerators employed in the vulcanization of rubber dolls and toys are usable, as

they have been devised to avoid the later presence of bad odors or bad tastes. The quantity used can be determined in accordance with the usual practices of correlating the quantity of rubber, sulphur and vulcanizing agent.

The paraffin, employed in the above example, was a refined paraffin wax having a melting point of 133 to 135° F. It is preferred to have a paraffin wax with a limited range of melting point: such materials are available in commerce from various sources, with trade specifications setting the range of melting point at 2 or 3 degrees F. In the above example, the paraffin wax employed at a specific gravity (solid at 60° F.) of 0.889 and (at 140° F. corrected to 60° F.) of 0.782; S. U. viscosity at 210° F. of 37/38; and was a refined crystalline type paraffin as distinguished from microcrystalline type. The quantity of paraffin can be varied from 10 to 40 parts, with corresponding variations of the behavior of the material. It is presently preferred to use a higher proportion of paraffin in making crown seals for soft drinks, and a lower proportion in making crown seals for beer. The paraffin operates to 25 restrict moisture vapor penetration, to restrict blocking, and to decrease any later leaching of materials from the composition by the action of some products which may be present in the container closed by the seal. The melting point of 30 the paraffin wax may be higher or lower, but it is presently preferred to have the melting point above normal atmospheric temperature conditions, and below the temperature at which the container may later be heated for pasteurization 35 or processing. When large proportions of wax are used, and a relatively sharp temperature transition is desired, it is preferred to employ paraffin waxes of the stated conventional type in distinction from microcrystalline waxes which 40 appear to have less compatibility with buna and natural rubbers than the conventional grades of paraffin wax, and in distinction from petrolatum waxes which have a relatively wide temperature range of softening; as these materials do not 45 behave so desirably as conventional paraffin waxes during the manufacture and use of the crown seals.

The titanium oxide and clay are fillers and also pigments. In the above example, the clay 50 and the titanium oxide were commercially available products widely used as inert fillers and pigments: other specific clays and forms of titanium oxide have been employed and are employable. With the indicated proportions of these fillers 55 and pigments, the resulting rubber film was substantially white in color. The ratio of fillers to one another may be varied in accordance with the color desired, and their total amount may be between about 200 parts and about 400 parts 60 per 100 parts of rubber base. These substances are illustrative of the general class of inert earthly fillers, and the various ochres, clays, barytes, etc. can be employed. The filler should be in finely divided condition, and preferably is 65 dense as distinguished from fluffy or spongy.

The composition can be blended on a rubber mill with means, such as an internal cold water flow, for keeping the rolls cool. The Buna rubber is milled with cold rolls for approximately 70 five minutes and then the zinc oxide and sulphur are added. When they have been incorporated in about five minutes time, the paraffin wax is added in the melted form: it is combined in about fifteen minutes. When this combination has been effected, the pigments are added and

combined. The vulcanizing agent is preferably added just before the rubber mass is to be coated or printed. Accordingly, the material can be made up in the absence of vulcanizing agent and diluent and stored for a considerable period without particular care. When it is to be used, the composition can be again rolled for incorporating the vulcanizing agent and then thinned with the diluent, or the stock mixture can be worked up with the diluent and the vulcanizing agent then incorporated, dependent upon the conditions for use.

The xylol is illustrative of diluent or fluidifying material, and its proportion may vary from 500 to 1000 parts, dependent upon the consistency of the printing which provides a deposit of uniform thickness without excessive flowing during the drying operation. It is preferred to bring the composition to liquid form by employing about 500 parts of the diluent xylol, and then introduce further diluent as necessary to bring the composition to proper viscosity for the printing operation. Other thinners can be employed, such as toluol or in general the volatile viscosity-reducing agents employed with rubbers: a true solvent action is not required as the function is to produce a mixture which will flow at the desired rate during printing.

In the above example, a thickness of individual deposit of about eight one-thousandths of an inch was set out. This thickness can be varied as desired, with a maximum thickness of about twelve one-thousandths of an inch. In practice, a dry thickness of fifteen one-thousandths of an inch total was produced by three coatings of the rubber compound, employing toluol as a thinner, representing three successive printings of five one-thousandths of an inch each with intervening drying operations.

The above illustration of practice describes a procedure of making a crown seal of the normal or standard size and shape, with manufacture from a blank having a diameter of one and one-half inch, with an annular deposit having a thickness of twenty-five one-thousandths of an inch, and a central or web thickness of eight one-thousandths of an inch. It has been found that, by employing the successional coatings, with forming and punching of shells and final vulcanization, satisfactory seals can be made with crown shells having a shorter skirt, and with employment of liner thicknesses of about fifteen one-thousandths of an inch. By comparison, it may be remarked that when cork composition is employed, the liner thickness is about 90 to 110 thousandths of an inch, which is compressed to about 30 thousandths of an inch as an incident of applying and crimping the crown seal.

In making a crown shell of the short skirt type, the printing operation may be conducted on the basis of blank diameters of  $1\frac{7}{8}$  inch, thus representing a saving of about 9% of the metal. Three deposits of composition, providing a total thickness of fifteen one-thousandths of an inch for the annular portion was employed, with a central web of five one-thousandths of an inch. These seals held excellently on standard bottle mouths and withstood the usual specifications with respect to internal pressure held with carbonated beverages. The thickness of a satisfactory sealing cushion is related to the total skirt depth; and the skirt edge should not be brought into interfering contact with the bottle neck during the operation of closing by crimping

while the cushion is under the prescribed compression pressure.

The application of the fluid composition may be accomplished by other than the silk screen method, such as employment of roller coating methods with the rolls having printing areas corresponding to the circles or rings at which deposit is to be made.

The GRS rubber is illustrative of a binding base used in admixture with filler and vulcanizing agent. Other macromolecular materials of elastically yielding type may be used. Such materials are prepared usually in mixture with filler and pigment such as clay and titanium oxide, thinned to suitable viscosity by an appropriate volatile agent such as xylol or toluol and then employed in the printing operation. Successive deposits, of limited thicknesses as set out above, are employed with drying of the diluent after each application, until a total thickness is built up to provide adequate yield for conforming to the irregularities at the container mouth to be sealed, these thicknesses being substantially those set out above for the rubber-paraffin mixtures. These deposits may be hardened individually, or as a group, by heating to the temperature at which curing by vulcanization, condensation or polymerization occurs, wherewith the product loses its original characteristic of being swollen or dissolved by the solvents, and of swelling by water.

The invention has been described above in illustrative practices. It will be understood that these are to indicate presently preferred conditions, and that the invention may be practiced in many ways within the scope of the appended claims.

We claim:

1. The method of making a crown closure, which comprises printing upon a sheet metal blank a succession of deposits of fluid material upon a predetermined area thereof corresponding to the internal end wall area of a crown shell, at least one of said deposits extending over the entire end wall area and at least one other of said deposits being restricted to the annular region at which the lip of the container engages the crown closure, said individual fluid material deposits comprising a volatile fluidifying substance and an elastically yieldable adherent material, the deposits being limited to produce after drying a maximum thickness per deposit of 0.012 inch and a maximum thickness of the total deposits of about 0.025 inch, drying off said volatile medium after each deposit and before the next deposit, and then forming the blank at parts radially outside the area into a container-engageable projecting flange with the deposits inside the same.
2. The method of making a crown closure, which comprises printing upon a sheet metal blank a succession of deposits of fluid material upon a predetermined area thereof corresponding to the internal end wall area of a crown shell, at least one of said deposits extending over the entire end wall area and at least one other of said deposits being restricted to the annular region at which the lip of the container engages the crown closure, said individual fluid material deposits comprising a volatile fluidifying substance and an elastically yieldable adherent material having a vulcanizable base and a vulcanizing agent, the deposits being limited to produce after drying a maximum thickness per deposit of 0.012 inch and a maximum thickness of the

total deposits of about 0.025 inch, drying off said volatile medium after each deposit and before the next deposit, then heating the blank to effect vulcanization of said material, and then forming the blank at parts radially outside the area into a container-engageable projecting flange with the deposits inside the same.

3. The method of making a crown closure, which comprises printing upon a sheet metal blank a succession of deposits of fluid material upon a predetermined area thereof corresponding to the internal end wall area of a crown shell, at least the first of said deposits extending over the entire end wall area and at least the last of said deposits being restricted to the annular region at which the lip of the container engages the crown closure, said individual fluid material deposits comprising a volatile fluidifying substance and an elastically yieldable adherent material, the deposits being limited to produce after drying a thickness per deposit of about 0.005 to 0.008 inch and a maximum thickness of total deposits of 0.015 to 0.025 inch, drying off said volatile medium after each deposit and before the next deposit, and then forming the blank at parts radially outside the area into a container-engageable projecting flange with the deposits inside the same.

4. The method of making a crown closure, which comprises printing upon a sheet metal blank a succession of deposits of fluid material upon a predetermined area thereof corresponding to the internal end wall area of a crown shell, at least the first of said deposits extending over the entire end wall area and at least two subsequent deposits being restricted to the annular region at which the lip of the container engages the crown closure, said individual fluid material deposits comprising a volatile fluidifying substance and an elastically yieldable adherent material, the deposits being limited to produce after drying a maximum thickness per deposit of 0.012 inch and a maximum thickness of total deposits of about 0.025 inch, drying off said volatile medium after each deposit and before the next de-

posit, and then forming the blank at parts radially outside the area into a container-engageable projecting flange with the deposits inside the same.

5. The method of making a crown closure, which comprises printing upon a sheet metal blank at each of a plurality of spaced predetermined regions on one side thereof a succession of deposits of fluid material, each said predetermined region including the internal end wall area of a crown shell, at least one of said deposits extending over the entire end wall area at each region and at least one other of said deposits being restricted to the annular part of each said region at which the lip of the container engages the crown closure, said individual fluid material deposits comprising a volatile fluidifying substance and an elastically yieldable adherent material having a vulcanizable base and a vulcanizing agent, the deposits being limited to produce after drying a maximum thickness per deposit of 0.012 inch and a maximum thickness of total deposits of about 0.025 inch, drying off said volatile medium after each deposit and before the next deposit, then heating the blank after the final deposit of said material thereon to effect vulcanization of said material, and then forming each said region of the blank at parts radially outside the corresponding said area into a container-engageable projecting flange with the corresponding deposits inside the same.

LOUIS F. ROGERS.  
MICHAEL S. EBERT.

## REFERENCES CITED

35 The following references are of record in the file of this patent:

## UNITED STATES PATENTS

| 40 | Number    | Name           | Date          |
|----|-----------|----------------|---------------|
|    | 1,734,847 | Bond           | Nov. 5, 1929  |
|    | 1,832,321 | Owens          | Nov. 17, 1931 |
|    | 1,901,682 | Warth          | Mar. 14, 1933 |
| 45 | 2,114,309 | McGowan et al. | Apr. 19, 1938 |